

## UNITED STATES PATENT OFFICE.

MELVIN W. BEARDSLEY, OF OAKLAND, CALIFORNIA.

## EXPLOSIVE AND PROCESS OF MAKING SAME.

SPECIFICATION forming part of Letters Patent No. 727,062, dated May 5, 1903.

Application filed January 5, 1903. Serial No. 187,907. (No specimens.)

*To all whom it may concern:*

Be it known that I, MELVIN W. BEARDSLEY, a citizen of the United States, residing at Oakland, in the county of Alameda and State of California, have invented a new and useful Improvement in Explosives and Processes of Manufacture, of which the following is a specification.

All explosives containing metallic salts of which the various chlorate-of-potash explosives may be taken as the type are more or less dangerous to handle and are liable also to deteriorate in strength and other qualities after their manufacture, especially when they are kept in a damp place or are exposed to moisture or extremes of temperature, and for the purpose of overcoming or removing the defects and objectionable features above mentioned various substances have been employed to cover the granules or particles of the mixture with a protecting coating of such an elastic nature that it will prevent physical contact of the metallic salts with one another and with the particles of the other ingredients, and in addition to acting as an isolating medium the substance so used will prevent the metallic salts from absorbing moisture.

My present improvement relates, chiefly, to the application, use, and combination in and with explosives of this class or description of the substances or product known as "corn-oil" to cover and protect the granules both from the effects of wet and moisture and also from physical contact and also to the production of an explosive possessing in a high degree the qualities of safety in manufacture, handling, and transportation, of retaining its strength and explosive properties under exposure to change of climate and extremes of temperature, and of being unaffected by dampness or moisture; and the invention is based on the discovery I have made that the product or substance known commercially as "corn-oil" is peculiarly adapted as a protecting medium or agent for the metallic salts and the particles of the other substances that enter as ingredients in these compounds or mixture. When mixed and incorporated with the particles or granules of the compound, it forms a protective coating that is permanently coherent, adhesive, and elastic, re-

taining its qualities and characteristics indefinitely and undergoing no change or deterioration under exposure to change of temperature or climate or lapse of time between the manufacture and the use of the explosive. It is, besides, rich in carbon in an advantageous form, being itself a hydrocarbon, and it is also found to simplify the process of manufacture of explosives of this class and to materially reduce their cost. Corn-oil combines readily with other liquid hydrocarbons, and particularly with the distillates of petroleum, thereby enabling the manufacturer of explosives containing metallic salts, carbon, and sulfur to vary their sensitiveness to detonation and explosion as may be required for specific purposes by the addition of such form of hydrocarbons in different proportions.

My invention therefore consists, essentially, in the application, combination, or mixture of the substance corn-oil in and with explosives containing metallic salts and in the improved production and manufacture of an explosive of high grade composed of a metallic salt, carbon, sulfur, and corn-oil, as hereinabove fully described, and set forth in the claims at the end of this specification.

Under the name of "metallic salts" I include the following substances: nitrate of potash, nitrate of soda, nitrate of barium, nitrate of ammonia, nitrate of lead, nitrate of lime, chlorate of potash, chlorate of ammonia, chlorate of soda, prussiate of potash, permanaganate of potash, picric acid, picrate of potash, picrate of ammonia, carbonate of magnesia. Under the name of "carbon" I include wood-charcoal, stone-coal, sugar, starch, charcoal made from peas or other leguminous seeds, charcoal made from rice, wheat, barley, corn, oats, or cotton-seed, wood-sawdust, the leaves of trees or plants dried and pulverized, wood-meal or wood-pulp, ground rice, wheat, oats, or barley chaff, wheat, oats, or barley bran, wheat, oats, barley, or rice flour or middlings, lampblack, and plumbago, and under the name of "sulfur" I include crude sulfur, refined sulfur, or sulfur in combination with any of its solvents, like sulfurated benzoin and the bisulfid of carbon.

In carrying out and applying my invention in the production of black gunpowder or black blasting-powder I add the corn-oil in about

- the proportion of eight per cent., by weight, to the other ingredients. A powder of this grade or quality is generally composed of nitrate of potash, nitrate of soda, sulfur, and charcoal in about the following proportions: nitrate of potash or soda, seventy-five parts; sulfur, ten parts; wood-charcoal, fifteen parts. After these substances are finely powdered and thoroughly dried the corn-oil is added first to the nitrate of potash or nitrate of soda and mixed and incorporated with its particles until each and every particle is thoroughly covered with the corn-oil. Then the charcoal is added and mixed with the coated and protected particles, and finally the sulfur is added and incorporated with the mass. The powder is now ready to be granulated by passing it through sieves, or it can be pressed into blocks of any shape or form desired. Any of the carbons hereinbefore mentioned may be employed instead of the charcoal for the purpose of changing the specific gravity of the finished powder or for the further purpose of increasing or diminishing its intensity. As the corn-oil is rich in carbon, I have found that seven per cent., by weight, of charcoal can be used instead of the quantity heretofore required in an explosive of the character made according to the foregoing formula, in which fifteen per cent. of charcoal is generally used. A gunpowder or a blasting powder produced from these ingredients with the addition of the corn-oil are found to possess several advantages over the ordinary powders or substances of the same class containing no corn-oil. They are not affected by exposure to atmospheric moisture and will not deteriorate rapidly when used for blasting in damp or wet ground. They are also much slower in their action when exploded, thereby reducing the breech-pressure in the case of gunpowder and rendering the blasting powder more useful for blasting coal or soft rock.
- In the manufacture of an explosive containing chlorate of potash the proportion of corn-oil can be varied to advantage. A good formula for an explosive compound of this character consists of chlorate of potash, eighty parts; sulfur, ten parts; wood-pulp, four parts; corn-oil, six parts. Any of the carbons hereinbefore mentioned can be used instead of wood-pulp, and for the same reasons as mentioned in connection with the manufacture of black powder the chlorate of potash being thoroughly dried and finely powdered the corn-oil is carefully and thoroughly incorporated with the chlorate until every granule or particle is fully covered by the oil. Then the sulfur is added and thoroughly incorporated with the oil-protected particles of chlorate, after which the carbon is added and thoroughly mixed with the mass. The powder is now ready to be granulated by passing it through sieves, or it may be pressed into blocks of any shape or size desired or loaded into paper or metallic shells. This chlorate-

of-potash powder is not affected by atmospheric moisture, and it can be stored for an indefinite period without undergoing deterioration in strength. It is a powerful explosive and will successfully rend hard rock. Another strong powder is made by mixing nitrate of soda or nitrate of potash with the chlorate of potash in the following proportions: chlorate of potash, forty-five parts; nitrate of soda or nitrate of potash, thirty parts; sulfur, ten parts; wood-charcoal, seven parts; corn-oil, eight parts. The process of mixing this powder is the same as that hereinbefore mentioned, it being borne in mind that the oil should first be mixed with the chlorate of potash. It will be evident to any one skilled in the art of explosives of this making, class, or description that the proportion of chlorate of potash to the nitrate of soda or potash can be varied to produce powders of different strength and sensitiveness, and I therefore only give the above formula as an example.

Another good and powerful explosive is produced by substituting nitrate of ammonia for the nitrate of soda or potash, as mentioned in the third formula; but in such case the nitrate of ammonia should be treated first with the corn-oil, as it is a "salt" that absorbs moisture readily and must be absolutely protected from exposure to atmospheric moisture, which can be done if the salts be properly mixed with the corn-oil.

In any or all of the explosive compounds embraced in the foregoing formulas the ingredient corn-oil will be found a great improvement over the various substances that have heretofore been used to secure protection of the metallic salts from moisture and to prevent premature explosion in compounds of this class, for the reason that it possesses the property of indefinitely retaining its elasticity and its coherent qualities unaffected by atmospheric conditions and temperature. It does not become brittle by oxidation or other causes. It forms a perfect "buffer" between the different substances in the composition of these explosives, thereby preventing any chemical action taking place in the compound and effectually preventing explosion by concussion. In these particulars it will be seen to differ from many hydrocarbons heretofore used for like purposes—such, for example, as coal-tar, wood-tar, pitch, asphaltum, or any of the distillates of petroleum.

I am aware that many vegetable oils have also been employed to accomplish the ends reached by me in the use of corn-oil; but I have learned by prolonged experiment that none of those which have been used in the production of high explosives of this class remain as constant or unchanged in their properties and characteristics as this substance, corn-oil.

All forms or varieties of explosive compounds containing corn-oil require to be fired

or detonated with a strong fulminate-of-mercury cap.

Having thus fully described my invention, what I claim as new therein, and desire to secure by Letters Patent, is—

1. An explosive compound composed of granules of oxygen-bearing metallic salts, carbon, sulfur and corn-oil.

2. An explosive compound composed of oxygen-bearing metallic salts, carbon and sulfur in the form of granules covered by a coating of corn-oil.

3. That improvement in the manufacture of explosives containing oxygen-bearing me-

tallic salts, consisting in reducing the salts to a fine powder then adding corn-oil in about the proportions specified and thoroughly incorporating the same so as to coat the granules, and afterward adding the carbon and sulfur previously pulverized, and mixing all the ingredients together.

In testimony whereof I have signed my name in the presence of two subscribing witnesses.

MELVIN W. BEARDSLEY.

Witnesses:

EDWARD E. OSBORN,

HARRY J. LASK.